

# UNITED STATES PATENT OFFICE.

EMIL GUSTAV STARK, OF ALTCHEMNITZ, NEAR CHEMNITZ, GERMANY.

## PROCESS OF TREATING BRITTLE VEGETABLE FIBERS OF KAPOK AND OTHER PLANTS.

1,023,890.

Specification of Letters Patent.

Patented Apr. 23, 1912.

No Drawing.

Application filed March 14, 1910. Serial No. 549,232.

To all whom it may concern:

Be it known that I, EMIL GUSTAV STARK, a subject of the German Emperor, and residing at Altchemnitz, near Chemnitz, Germany, have invented a certain new and useful improved process of treating brittle vegetable fibers of kapok and other plants for uniformly dyeing, spinning, and working them into yarn and twine, of which the following is a specification.

My invention relates to processes for the treatment of a number of vegetable fibers, particularly the down or hair of the seed, of kapok (*Eriodendron anfractuosum*), *Calotropis procera*, pseudo-china, cotton silks, acundha, and, indeed, all the fibers, *i. e.* the hair of the seed, of the group of *Asclepias*, and the like, most of which are designated cotton silks, have a beautiful brilliant appearance, and are brittle in their natural condition, so that they cannot be spun.

A primary object of my invention is to provide a process which enables these vegetable fibers, *i. e.* the hair of the seed, to be spun.

According to my process the smooth surface of the vegetable fibers, treated with suitable solvents, is shrunk and converted into a rough surface. When treating the vegetable fibers with the solvents those substances are simultaneously removed from the vegetable fibers which cause the brittleness of the fibers. These are incrusting substances both of inorganic and organic nature. The solvent is caused to act on the fibers until the incrusting substances have for the most part passed into the solvent. The solvents can act at an ordinary temperature on the vegetable fibers, but in order to accelerate the treatment, I prefer to heat them.

When aqueous solvents are employed, I may add coloring-matter to the solvent in order to dye the vegetable fibers.

My process characterized above by its general principal features may be carried into practice in various ways according to the solvents selected in each instance. For example, the incrusting substances may be removed from the vegetable fibers by extraction by means of a dilute aqueous solution of glue, preferably at a temperature of 60° C. to nearly 100° C. according to the nature of the fibers in each instance. Also, a very small admixture of alkali is preferable in

individual instances, when the last mentioned solution is employed, according to the nature of the vegetable fibers in each instance. The above mentioned solution can be recovered and utilized repeatedly. When the vegetable fibers are treated with aqueous solutions of glue it is preferable previously to macerate the vegetable fibers with dilute tannin-liquor, because the fibers thereby obtain increased strength.

The vegetable fibers liberated from the incrusting substances are washed in water and then dried at a moderate temperature. The same are then adapted to be uniformly dyed, spun and worked up by themselves or with other vegetable fibers into yarn and twine.

Obviously my new process is not only applicable for the vegetable fibers named above, but also for those vegetable fibers which possess similar qualities as the fibers, *i. e.* the hair of the seed, of kapok (*Eriodendron anfractuosum*) and cotton silks generally.

I claim:

1. The herein-described process of treating brittle vegetable fibers, *i. e.* the down or hair of the seed, of kapok (*Eriodendron anfractuosum*), *Calotropis procera*, pseudo-china, cotton silks, acundha, and of the group of *Asclepias* and the like, most of which are designated cotton silks, which consists in treating the fibers with a dilute, aqueous solution of glue, thereby dissolving a portion of the incrusting substances within the single hair, extracting the same therefrom and thereby shrinking the smooth surface of the fibers and converting it into a rough surface.

2. The herein-described process of treating brittle vegetable fibers, *i. e.* the down or hair of the seed, of kapok (*Eriodendron anfractuosum*), *Calotropis procera*, pseudo-china, acundha, and of the group of *Asclepias* and the like, most of which are designated cotton silks, which consists in treating the fibers with a dilute, slightly alkaline, aqueous solution of glue, thereby dissolving a portion of the incrusting substances within the single hair, extracting the same therefrom and thereby shrinking the smooth surface of the fibers and converting it into a rough surface.

3. The herein-described process of treating brittle vegetable fibers, *i. e.* the down or hair of the seed, of kapok (*Eriodendron*

unfractuosum), *Calotropis procera*, pseudo-china, cotton silks, acundha, and of the group of *Asclepias* and the like, most of which are designated cotton silks, which 5 consists in macerating the fibers with dilute tannin-liquor, and subsequently treating them with an aqueous solution of glue and thereby dissolving a portion of the incrusting substances within the single hair, extracting the same therefrom and thereby 10 shrinking the smooth surface of the fibers and converting it into a rough surface.

4. The herein-described process of treating brittle vegetable fibers, *i. e.* the down or 15 hair of the seed, of kapok (*Eriodendron anfractuosum*), *Calotropis procera*, pseudo-china, cotton silks, acundha, and of the group of *Asclepias* and the like, most of which are designated cotton silks, which 20 consists in treating the fibers with an aqueous solution of glue containing color-

ing matter thereby dissolving a portion of the incrusting substances within the single hair, extracting the same therefrom and thereby shrinking the smooth surface of 25 the fibers and converting it into a rough surface.

5. The herein-described process of treating brittle vegetable fibers of the character described, which consists in removing therefrom by means of an aqueous solution containing coloring matter, the adhering, incrusting substances and thereby shrinking the smooth surface of the fibers and converting it into a rough surface. 30

In testimony whereof I affix my signature in the presence of two witnesses.

EMIL GUSTAV STARK.

Witnesses:

WILLIAM J. KOUJETSUY,  
M. F. BENNDORF.